

1

2,820,008

## LUBRICATING GREASE COMPOSITION

Harold A. Woods and Harvey M. Trowbridge, Martinez, Calif., assignors to Shell Development Company, New York, N. Y., a corporation of Delaware

No Drawing. Application April 22, 1955  
Serial No. 503,340

9 Claims. (Cl. 252—33.3)

This invention is concerned with improved grease compositions. More particularly, it is directed to grease compositions conferring markedly improved corrosion protection and bearing life, and having greater mechanical stability.

Grease compositions comprising a lubricating oil and soap are subject to two primary degrading influences, namely, oxidation and the deleterious effects of products produced thereby, as well as due to thermal degradation and the resulting decomposition products thereof. A great variety of additive materials have been studied for their effect upon the several properties of greases such as maintenance of consistency, depression of corrosion characteristics, stabilization against oxidation and resistance to thermal decomposition. One property which most greases are subject to in addition to those discussed above is the sensitivity of the composition with respect to water. Most soaps and therefore soap-based greases are sensitive to a lesser or greater degree to emulsification or solution in water. Since wheel bearings and similar lubrication points are subject to the washing action of water especially in wet weather it is imperative that greases be constructed so as to be resistant to excessive emulsification or solution thereof in water or similar solvents.

In addition to the sensitivity of a grease with respect to water, other situations occur in which the machinery to be lubricated is subject to corrosive agents such as organic acids and the like. Such is the case in cannery equipment, an aggravated example of which is equipment utilized for the canning or freezing of spinach and similar vegetables. Many food juices, such as spinach juice are corrosive to metal. In addition, they are often preserved in weak brines. The combination of the food juices and the brines is often extremely corrosive to the equipment. Consequently, greases must be designed to protect cannery equipment from corrosion, especially for the processing of such materials.

It is an object of the present invention to provide greases especially suitable for operation of machinery in the presence of water. It is another object of the present invention to provide grease compositions which will afford protection against corrosion by aqueous brine and food juices such as those just described. It is a further object of the present invention to provide grease compositions not only improved in the two respects just mentioned but also having greatly prolonged mechanical stability. Other objects will become apparent during the following discussion.

Now, in accordance with the present invention, soap base greases comprising a major amount of a lubricating oil thickened to a grease consistency with a minor proportion of a metallic soap have been unexpectedly improved by the synergistic combination of mono (aliphatic carboxylic acid) esters of polyoxyalkylene glycols (wherein each oxyalkylene radical contains 2-6 carbon atoms) and alkaline earth metal hydrocarbyl sulfonates. It has been found that the combination of these particular additives, especially when they are present in amounts each of be-

2

tween about 0.1% and about 5%, by weight, based on the total grease composition, provides an unexpected prolongation in the useful bearing life of the grease, are unexpectedly resistant to the washing or emulsification action of water, and provide excellent resistance against corrosion for metallic surfaces lubricated thereby.

The polyalkylene glycol monoesters have the general formula

10



wherein R is an alkylene radical having between about 2 and about 6 carbon atoms, preferably between 2 and 4 carbon atoms. R<sub>1</sub> is an alkyl radical having between about 8 and about 24 carbon atoms, preferably between about 12 and about 20 carbon atoms, and n is a whole integer between about 5 and about 20. Preferably the polyoxyalkylene glycols from which the subject monoesters are formed have molecular weights between about 150 and about 2000, and the monoesters derived therefrom are of high enough molecular weight to be oil-soluble. Suitable glycols from which the monoesters may be prepared include polyethylene glycol, polypropylene glycol, polybutylene glycol, polyamylene glycol, and polyhexylene glycol, as well as combinations thereof including the heteric polymers of ethylene glycol and propylene glycol, for example. Acids which may be utilized in accordance with the present invention to form the subject monoesters comprise both saturated and unsaturated aliphatic monocarboxylic acids, including both fatty acids and hydroxy fatty acids. Included expressly are capric, lauric, myristic, palmitic, and stearic acids, and the corresponding unsaturated acids of which oleic acid is typical and preferred. Also the corresponding hydroxy fatty acids may be utilized such as 12-hydroxy stearic acid, or the corresponding mixtures derived by the hydrogenation of castor oil or similar naturally occurring oils. Typical species of suitable monoesters comprise the oleic acid esters of polyethylene glycol, the stearic acid esters of polypropylene glycol, polyethylene glycol monolaurate, and the like.

The alkaline earth metal hydrocarbyl sulfonates are preferentially oil-soluble and preferably are obtained from petroleum sources and are known as petroleum sulfonates. These are ordinarily obtained in the treatment of petroleum oils to obtain highly refined products of the type of electrical insulating oils, turbine oils and the like, in which the petroleum oils are treated successively with a number of portions of concentrated sulfuric acid or fuming sulfuric acid. A variety of compounds are formed by the chemical reactions of sulfuric acid upon the oil including sulfonic acid, organic esters of sulfuric acid, partial esters of sulfuric acid, etc. Most of these compounds are relatively insoluble in the oil under the treating conditions and separate from the oil together with unreacted sulfuric acid as a sludge, which is separated from the oil after each treatment. The sulfuric acid is usually added in "dumps" of about 1/2 lb. per gallon of the oil, the total quantity of the acid added depending upon the oil being treated and the desired final product. Usually from about 3 pounds to about 9 pounds of sulfuric acid per gallon of oil are used. Some of the sulfonic acids resulting from the treatment of the oil with the sulfuric acid are preferentially oil-soluble and remain in the oil layer after removal of the acid sludge. These can be removed from the oil by neutralizing the acid-treated oil with an alkaline agent such as oxides, hydroxide, or carbonate of an alkaline earth, for example, calcium oxide, to form sulfonic acid soaps or sulfonates which are then extracted from the oil by treatment with 50% to 80% aqueous alcohol solutions or other suitable means. Because of the

characteristic mahogany color of the sulfonates they are known in the petroleum art as mahogany soaps. While the majority proportions of the preferentially oil-soluble sulfonates are obtained from the acid-treated oil, there can be recovered from the acid sludge by suitable solvents preferentially oil-soluble sulfonates or sulfonic acids. The term "preferentially oil-soluble" sulfonates therefore includes the oil-soluble sulfonates from both the acid-treated oil and the acid sludge. Preferably the sulfonic acids have molecular weights in the order of about 400 to 750.

The alkaline earth metal salts or soaps of the subject sulfonic acids may be either the so-called neutral soaps wherein all of the hydroxyl groups of the neutralizing agent such as lime are combined with sulfonic acid radicals, or the so-called basic sulfonates may be employed wherein the metallic radical has one valence attached to a sulfonic acid radical and the other being a hydroxyl substituent.

The preferred sulfonates are the so-called "basic sulfonates," believed to have the general formula represented by



wherein R is a hydrocarbyl radical, M is an alkaline earth radical, R usually being a naphthyl, alkyl naphthyl, alkaryl or naphthyl aryl radical, such that the weight of the sulfonic acid is that stipulated hereinbefore. The possibility exists that the basic sulfonate comprises a colloidal mixture of the neutral sulfonate and alkaline earth metal hydroxide.

The soap greases to be benefitted by the presence of this combination of improving substances comprise those wherein the lubricating oil is of mineral oil origin or of synthetic origin as given in greater detail hereinafter. The soaps utilized for thickening these oils to a grease consistency comprise the alkali metal or alkaline earth metal soaps of fatty acids or hydroxy fatty acids, including especially the calcium- or lithium soaps of stearic acid or of 12-hydroxy stearic acid. Other soaps utilized for the formation of suitable greases to be included within the present invention are well known in the art. Calcium and lithium stearates or hydroxy stearates have a certain amount of inherent water resistance and are preferred for this reason. However, the invention contemplates the use of more water-sensitive soaps as well, such as the sodium soaps of suitable fatty acids. The fatty (or hydroxy fatty) acids which may be employed are those having between about 12 and about 24 carbon atoms per molecule, preferably between about 16 and 20 carbon atoms per molecule. Ordinarily, sources of acids are utilized which preponderate in acids having an average of about 18 carbon atoms per molecule such as those obtained from castor oil or from animal fats, and the like.

In addition to the ordinary mineral oils utilized as is known in the art for the preparation of greases, synthetic lubricants may be utilized including the aliphatic esters of dicarboxylic acids, the liquid polyoxyalkylene glycols and oxides, liquid phosphorus esters, silicates, and similar materials. Typical species of these classes include tricresyl phosphate, tri(2-ethylhexyl) phosphate, bis(2-ethylhexyl) sebacate, adipate, tetrahexyl silicate, heteric copolymers of ethylene oxide and propylene oxide, and similar substances.

One of the unexpected features of the present invention comprises the very substantial increase in the mechanical stability of the greases containing the recited combination of additive substances. This is especially unexpected in view of the fact that the single substances utilized in the absence of the other even in the same type of grease compositions results in no increase in roll stability or at least in an improvement of only a minor amount. This feature is especially evident in Example I given hereinafter, and the effect is most pronounced at elevated temperature, in the order of at least about 150° F. and above. Even at room temperature, however, it has been found that the use of the combination of

additives results in substantially doubling the effective life of the grease composition under mechanical stress.

In studying the various possible aspects of the general class of compositions considered herewith, the use of the corresponding sodium sulfonates was considered. However, as the comparative data given in Example I demonstrates, the alkali metal sulfonates are highly undesirable, since when utilized in amounts effective to promote even a mild degree of corrosion protection in the grease compositions, their presence creates a substantial amount of water sensitivity as evidenced by the percent of the grease lost by means of emulsification or otherwise in a standard water resistance test. As the proportion of sodium sulfonate is increased for the purpose of providing further protection against corrosion, the water resistance of the grease drastically decreases. Thus, by increasing the proportion of sodium sulfonate from about 2% to about 2½% in the same lithium 12-hydroxy-stearate-mineral oil grease, the percent loss of grease in a water resistance test increased from 32% to about 55%. Thus it was determined that sodium sulfonates could not be used in the present compositions due to their disadvantageous tendency to create water sensitivity of the grease. For this reason, as well as because of the superior mechanical stabilizing properties of the alkaline earth metal sulfonates, the alkali metal sulfonates are not included within the scope of the present invention.

#### Example I

| 30                                                                     | Water washout, percent loss | 14 days' glass jar corrosion test—0.05% NaCl—number of rollers corroded | Hours to 230 per roll stability |            |
|------------------------------------------------------------------------|-----------------------------|-------------------------------------------------------------------------|---------------------------------|------------|
|                                                                        |                             |                                                                         | 212° F.                         | Room temp. |
| 35                                                                     |                             |                                                                         |                                 |            |
| Base grease +2% Na sulfonates +2.5% poly(ethylene glycol) mono-oleate  | 32                          | 4                                                                       | 48                              | 300        |
| 40 Base grease +2% Ca sulfonates +2% poly(ethylene glycol) mono-oleate | 11                          | None                                                                    | 290                             | 550        |
| Base grease                                                            | 5                           | 12                                                                      | 36                              | 300        |

The "base grease" employed in the above example comprised the lithium 12-hydroxystearate soap in gelling amounts and a medium viscosity mineral lubricating oil in a major amount.

Further investigation of the subject grease compositions disclosed the fact that the combination of monoesters and alkaline earth metal sulfonates, while providing a highly unexpected increase in the mechanical stability of the grease, at the same time caused the grease to become somewhat more sensitive to oxidation. While this property is of no importance when the grease is utilized in applications where attacked by oxygen is of a minor order, it would be highly desirable to overcome this property if it is possible to do so. The further preparation of polyvalent metal salts of dithiocarbamic acid has been found to not only restore the original stability of the grease but actually can cause an unexpected increase in the oxidation resistance thereof. Typical members of this class of additives comprise the zinc, aluminum, lead, iron, calcium, barium, and sodium salts of dialkyldithiocarbamates such as the zinc salt of dibutyl-dithiocarbamate, the calcium salt of diethylidithiocarbamate, the barium salt of dimethylidithiocarbamate, the lead salt of dimethylidithiocarbamate, the zinc salt of dihexylidithiocarbamate, the barium salt of diamylidithiocarbamate, and the corresponding salts of dioctyl dipropyl, propyl, butyl and ethylphenyl dithiocarbamate. These materials should be utilized in an amount between about 0.01 and about 1.5% by weight of the total grease composition.

As Example II given below shows, the use of the zinc dibutylidithiocarbamate not only restored the oxidation

stability of the grease composition after it had been somewhat degraded in this respect by the addition of the combined calcium petroleum sulfonate and polyethylene glycol monooleate, but actually improved the composition in this property.

*Example II*

|                                                                            | No. 1 | No. 2 | No. 3 |
|----------------------------------------------------------------------------|-------|-------|-------|
| Composition, percent weight:                                               |       |       |       |
| Base grease                                                                | 100   | 96.0  | 95.5  |
| Poly(ethyleneglycol) monooleate                                            |       | 1.0   | 1.0   |
| Calcium petroleum sulfonates <sup>1</sup>                                  |       | 3.0   | 3.0   |
| Zinc salt of dibutyl dithiocarbamate                                       |       |       | 0.5   |
| Navy EES bearing test: (250° F., 10,000 R. P. M.), time for failure, hours | 653   | 483   | 925   |

<sup>1</sup> 33.3% concentrate.

Still further improvements may be made by the addition of other types of ingredients such as aromatic amines including the phenyl-alpha-naphthylamine and other naphthylamines as well as guanadine derivatives and the like.

The invention claimed is:

1. A grease composition comprising a mineral lubricating oil thickened to a grease consistency with an alkali metal soap of a hydroxy fatty acid having from 12 to 24 carbon atoms per molecule and between about 0.25% and about 5% by weight each of an oil-soluble alkaline earth metal basic sulfonate and a mono(unsaturated fatty acid) ester of a polyalkylene glycol said glycol having 5-20 alkylene radicals, said fatty acid having from about 12 to about 24 carbon atoms per molecule.

2. A grease according to claim 1, containing in addition from about 0.01% to about 5% by weight of an oil soluble zinc salt of a dialkyl dithiocarbamate.

3. A grease according to claim 1, containing in addition from about 0.01% to about 5% by weight of an oil-soluble metal salt of a dialkyl dithiocarbamic acid.

4. A grease composition comprising a major amount of a mineral lubricating oil thickened to a grease consistency with a minor amount of lithium soap of 12-hydroxystearic acid, and from about 0.25% to about 5% by weight each of basic oil-soluble calcium petroleum sulfonates and a polyethylene glycol mono-oleate said glycol having 5-20 ethylene radicals.

5. A grease composition according to claim 4 containing in addition between about 0.1% and about 5% by weight of zinc dibutyl dithiocarbamate.

6. A grease composition comprising a major amount of a mineral lubricating oil, a minor proportion sufficient to thicken said oil to grease consistency of an alkali metal soap, and between about 0.25% and about 5% by weight each of an oil-soluble alkaline earth metal

basic sulfonate and a mono fatty acid ester of a polyalkylene glycol said glycol having 5-20 alkylene radicals, said fatty acid having from about 12 to about 24 carbon atoms per molecule.

5 7. A grease composition comprising a major amount of a mineral lubricating oil, a minor proportion sufficient to thicken said oil to a grease consistency of an alkali metal soap and between about 0.25% and about 5% by weight each of an oil-soluble alkaline earth metal petroleum sulfonate and a polyalkylene glycol monoester having the general formula



10 15 wherein  $n$  is an integer between 5 and 20, R is an alkylene radical having 2-6 carbon atoms and  $R_1$  is an aliphatic hydrocarbon radical having 8-24 carbon atoms.

8. A grease composition comprising a major amount of a mineral lubricating oil, a minor proportion sufficient to thicken said oil to a grease consistency of an alkali metal soap, and between about 0.25% and about 5% by weight each of an oil-soluble alkaline earth metal hydrocarbyl sulfonate and a polyalkylene glycol monoester having the general formula



25 30 wherein  $n$  is an integer between 5 and 20, R is an alkylene radical having 2-6 carbon atoms and  $R_1$  is an aliphatic hydrocarbon radical having 8-24 carbon atoms.

9. A grease composition comprising a major proportion of a lubricating oil, a minor proportion, sufficient to thicken said oil to a grease consistency, of a soap of the group consisting of alkali metal fatty acid soaps, alkaline earth metal fatty acid soaps, alkali metal hydroxy fatty acid soaps and alkaline earth metal hydroxy fatty acid soaps, and between about 0.25% and about 5% by weight each of an alkaline earth metal hydrocarbyl sulfonate and a polyalkylene glycol monoester having the general formula



35 40 45 wherein  $n$  is an integer between 5 and 20, R is an alkylene radical having 2-6 carbon atoms and  $R_1$  is an aliphatic hydrocarbon radical having 8-24 carbon atoms.

References Cited in the file of this patent

UNITED STATES PATENTS

- Re. 23,243 Bondi \_\_\_\_\_ June 20, 1950  
 2,352,811 Swenson \_\_\_\_\_ July 4, 1944  
 2,450,633 Clayton \_\_\_\_\_ Oct. 5, 1948